

Jan. 9, 1945.

F. G. PELLETT

2,367,047

MICA SHEET AND PROCESS FOR MAKING THE SAME

Filed Feb. 18, 1941



Inventor:  
Fred G. Pellett,  
by *Harry E. Dimkans*  
His Attorney

## UNITED STATES PATENT OFFICE

2,367,047

MICA SHEET AND PROCESS FOR MAKING  
THE SAME

Fred G. Pellett, Alplaus, N. Y., assignor to General Electric Company, a corporation of New York

Application February 18, 1941, Serial No. 379,541

2 Claims. (Cl. 154—2.6)

This invention relates to articles comprising bonded mica flakes or fragments. It is particularly concerned with the surfacing of such articles with thin, smooth coatings of a thermoplastic resin such as a methacrylate resin.

Because natural mica cannot be obtained readily in sheets of suitable area and thickness, electrically insulating mica sheets ordinarily comprise comparatively small mica flakes bonded together by means of a suitable binder. Copal resins, alkyd resins and, in particular, shellac have been widely used as organic binders therefor. In accordance with the usual practice, the individual mica flakes are coated with a thin film of the binder, for example, from a solution thereof, are then dried to remove the solvent and are thereafter assembled in such a manner that upon pressing between hot parallel press plates an insulating sheet of considerable area is obtained. Due to the shape of the individual mica fragments, very little flowing or slippage thereof takes place during the pressing operation so that with the process generally used for arranging and coating the flakes prior to pressing, pressed sheets of non-uniform or uneven thickness are ordinarily obtained. As most electrical applications require insulating sheets of a more uniform thickness, the surface of these pressed mica sheets are usually sanded or otherwise surface finished to obtain a product of uniform thickness. This surface-finishing of the sheet results in the exposure of mica flakes which are no longer coated with the binder and which tend to flake off or feather. Such sheets or segments cannot be used, for example, in the assembly of commutators by means of automatic machines. Their sanded surfaces are not particularly slippery and the mica edges may catch on the loosened or feathering fragments on the surfaces of the adjacent pieces, thus preventing automatic handling of the segments by the machine.

It previously has been proposed to resurface the sanded sheets with a material such as shellac, but as this practice is not adaptable to hot pressing, an entirely satisfactory finish is not obtained in that the resultant surfaces are not very smooth or slippery nor are they entirely free from a tendency towards flaking of the mica. It has also been proposed to surface bonded mica sheets with thin sheets of chemically treated cellulose such as cellulose acetate. However, the thinnest sheets of such material commercially available produce a marked over-all increase in the organic content of the mica insulating material which is obviously undesirable where for electrical reasons

the maximum possible amount of mica per unit volume of insulating material is desired. Furthermore, it has been found that in punching mica sheets surfaced with chemically treated cellulosic sheet materials there is some tendency for the cellulose layers to separate from the underlying mica layer with the production of frayed or delaminated edges obviously as undesirable in the final product as are the feathery surfaces of the uncoated sanded sheets.

An object of the present invention is to overcome and eliminate the above defects by providing mica sheets having thin firmly-adhering surface coatings of a non-sticking material which will not materially increase the total organic content of the sheets.

Another object of the invention is to provide mica sheets with a surfacing material which can be applied from solution and the coated sheets thereafter hot pressed to produce a smooth flat surface thereon.

Other objects of the invention will become apparent from the following description of the invention taken in connection with the accompanying drawing in which the single figure is a perspective view of a mica sheet provided on both sides with the surfacing material in accordance with my invention.

Of all the numerous coating materials tried, the methacrylate resins, i. e., the polymerized esters of methacrylic acid such as polymethyl-methacrylate, were the only ones found capable of meeting all of the above-mentioned objects.

In accordance with my invention, the mica flakes or fragments which have previously been coated with a suitable binder such as shellac are thereafter assembled and hot pressed into the form of a laminated mica sheet in accordance with the well known practice. The pressed sheet is sanded to the desired thickness and the sanded sheets are coated with a thin film of methacrylate resin as from a suitable solution thereof. An example of a suitable coating composition is one of the following composition:

|                           | Per cent |
|---------------------------|----------|
| Methyl methacrylate resin | 8        |
| Montan wax                | 0.75     |
| Toluol                    | 91.25    |

The mica sheets may be coated with this solution using ordinary coating rollers. However, any other convenient method may be used such as brushing or dipping. After the solvent has evaporated the coated sheets are hot pressed between smooth steel press plates to obtain the finished product.

The montan wax called for in the above formula acts as a lubricant during the pressing of the coated sheets. It is to be understood that other lubricants may be used or the lubricant may be omitted from the coating formula and applied instead directly to the press plates. Solvents other than toluol may be used and the concentration of the solution may be varied to suit the coating method or to obtain the desired film thickness.

Preferably in order to keep the organic content of the finished sheets as low as possible, the coating solution should be rather dilute. For practical applications, the concentration thereof should not exceed approximately 20 per cent. The calculated film thickness of the surface film obtained with the above-mentioned 8 per cent methacrylate composition averages about 0.00009 inch. With a 30 mil mica sheet containing approximately 5 per cent binder, which is the average binder content of bonded mica segments for small commutators, the application of such thin films of the methyl methacrylate resin adds about 0.25 per cent organic material to the sheet representing approximately a 5 per cent increase in total content of organic material. Preferably, the surface films of methacrylate resin should not exceed substantially 0.0001 inch in average thickness. An outstanding advantage of the methacrylate surface coatings results from the fact that the sheets coated therewith may be hot pressed without sticking to the heated press plates. Hot pressing produces a much smoother surface than cold pressing. There is also a marked reduction in the tendency for mica to split or flake at the

edges of the sheets or segments during punching and handling when surfaced with the methacrylate resins.

Although the surfaced sheets of my invention are suitable for use wherever laminated mica sheets have previously been used, they are particularly adapted, as has previously been stated, in the machine assembly of small commutators where it is essential that the small segments readily slide one over the other without the mica edges thereof tending to catch on the surfaces of the adjacent mica segments or on parts of the machine. There is no tendency for the methacrylate coated sheets to adhere to one another in the machine under ordinary summer heat and pressure conditions.

What I claim as new and desire to secure by Letters Patent of the United States is:

1. An article of manufacture comprising a composite sheet of shellac-bonded mica flakes sanded to uniform thickness, the said sanded sheet having a thin, smooth surface coating of a methacrylate resin not exceeding substantially 0.0001 inch in average thickness intimately bonded thereto.
2. The process of making a composite mica sheet for use in the machine assembly of commutator segment insulation which comprises hot pressing shellac-coated mica fragments into sheet form, sanding the pressed sheet to desired thickness, applying a dilute solution of a methacrylate resin to the surfaces of said sanded sheet, permitting the solvent to evaporate and again hot pressing the coated sheet.

FRED G. PELLETT.